

Jan. 13, 1925.

1,523,005

J. H. DORAN

NOZZLE DIAPHRAGM HAVING CAST IN NOZZLE PARTITIONS AND METHOD OF  
MANUFACTURING THE SAME  
Filed May 9, 1922

Fig.1.



Fig.2.



Inventor:  
John H. Doran,  
by *John H. Doran*  
His Attorney

## UNITED STATES PATENT OFFICE.

JOHN H. DORAN, OF SCHENECTADY, NEW YORK, ASSIGNOR TO GENERAL ELECTRIC COMPANY, A CORPORATION OF NEW YORK.

NOZZLE DIAPHRAGM HAVING CAST-IN NOZZLE PARTITIONS AND METHOD OF MANUFACTURING THE SAME.

Application filed May 9, 1922. Serial No. 559,680.

*To all whom it may concern:*

Be it known that I, JOHN H. DORAN, a citizen of the United States, residing at Schenectady, in the county of Schenectady, State of New York, have invented certain new and useful Improvements in Nozzle Diaphragms Having Cast-In Nozzle Partitions and Methods of Manufacturing the Same, of which the following is a specification.

The present invention relates to nozzle diaphragms for elastic fluid turbines, especially nozzle diaphragms of the type in which the nozzle partitions are cast into the diaphragms, and has for its object to provide an improved structure of diaphragm and an improved method of manufacturing the same.

For a consideration of what I believe to be novel and my invention, attention is directed to the following specification and the claims appended thereto.

In the drawing, Fig. 1 is a side elevation of a diaphragm structure embodying my invention, and Fig. 2 is a radial sectional view thereof.

Diaphragms are usually made in upper and lower halves for purposes of assembling, and in the drawing I have illustrated a half diaphragm. It will be understood, however, that my invention may be carried out in connection with diaphragms cast in halves or as a whole.

Both cast steel and cast iron have been used in the manufacture of diaphragms having cast-in nozzles. Cast steel is particularly satisfactory so far as strength of the material is concerned but it offers difficulties in that during the casting it is quickly chilled by the nozzle partitions and does not make a good joint with them. In other words, it is difficult to cast the nozzle into steel. On the other hand, nozzle partitions are easily cast into cast iron, but this material is not so satisfactory as steel because it is not so strong. The greatest stresses in a diaphragm occur in the vicinity of the hub and the use of cast iron requires rather thick, heavy diaphragms in order to give the necessary strength to the diaphragms.

Now, according to my invention, I construct a diaphragm in which the outer or

peripheral portion which holds the nozzle partitions is made of cast iron and the inner or web portion is made of cast steel, the two parts being joined together by an interlocking joint which may be somewhat of the nature of a tongue and groove connection. In carrying out my invention, I form the mold for casting the diaphragm in any usual or desired manner, mounting the nozzle partitions therein in the customary way. Then at a point spaced radially inward from the nozzle partitions I arrange in the mold a separator formed of a strip of suitable metal reversely bent on itself to form deep corrugations or pockets into which the molten iron and molten steel can flow. In the drawing, 5 indicates the nozzle partitions, 6 the cast iron part of the diaphragm, 7 the cast steel part of the diaphragm, and 8 the separator bent to provide pockets 9 and 10, which receive iron and steel respectively. The separator is made of suitable width so it is supported in the sand of the mold and after the diaphragm is cast the edges projecting beyond the surfaces of the diaphragm are removed.

The iron and steel parts of the diaphragm are poured preferably at the same time or about the same time so that they both cool and harden simultaneously. On account of the difference in pouring temperatures of steel and iron, steel being poured at a higher temperature than iron, the steel may be poured first, and after it has cooled a predetermined amount, the iron poured. Upon hardening the iron and steel parts of the diaphragm are firmly joined together.

While I have particularly described my invention as relating to nozzle diaphragms and its use with the metals steel and iron, it will be understood that my invention in its broader aspects is not necessarily limited to this particular use, but may be utilized whenever found applicable and with such metals as desired.

What I claim as new and desire to secure by Letters Patent of the United States, is:

1. A nozzle diaphragm for a turbine having its peripheral portion formed of cast iron and its web portion of cast steel.
2. A nozzle diaphragm for a turbine hav-

ing the part which holds the nozzle partition formed of cast iron and the remainder of cast steel.

3. A nozzle diaphragm for a turbine having its radially outer portion formed of one metal and its radially inner portions formed of a different metal, said portions being joined by an interlocking joint.

4. A nozzle diaphragm for a turbine having its radially outer portion formed of one metal and its radially inner portion formed of a different metal, said portions being joined by a tongue and groove connection.

5. The method of manufacturing a nozzle diaphragm having its peripheral portion formed from one metal and its web portion from another metal, which comprises arranging the nozzle partitions and a separator in a mold and then pouring the two metals which are to form the diaphragm.

6. The method of manufacturing a nozzle diaphragm having its peripheral portion formed from one metal and its web portion from another metal, which comprises arranging the nozzle partitions and a deep-

ly corrugated separator in a mold and then pouring the two metals which are to form the diaphragm.

7. A composite structure cast from metals and having one portion cast from one metal and another portion cast from another metal, the two portions being joined by a tongue and groove connection comprising a strip which is reversely bent on itself to provide oppositely-facing pockets which are filled with the respective metals.

8. The method of manufacturing a cast composite structure having a portion formed of one metal and a second portion formed of another metal which comprises arranging a separator in the mold, said separator comprising a strip reversely bent on itself to provide oppositely facing pockets, and pouring the metals to form the respective portions, whereby the metals will flow into the pockets to join the portions together.

In witness whereof, I have hereunto set my hand this 8th day of May 1922.

JOHN H. DORAN.